

# UNITED STATES PATENT OFFICE.

RICHARD GEORGE WOODBRIDGE, JR., OF WILMINGTON, DELAWARE, ASSIGNOR TO  
E. I. DU PONT DE NEMOURS & COMPANY, OF WILMINGTON, DELAWARE, A CORPO-  
RATION OF DELAWARE.

## PROCESS OF MAKING PROPELLENT POWDER.

1,379,073.

Specification of Letters Patent.

Patented May 24, 1921.

No Drawing.

Application filed August 8, 1919. Serial No. 316,030.

To all whom it may concern:

Be it known that I, RICHARD GEORGE WOODBRIDGE, Jr., a citizen of the United States, and a resident of Wilmington, in the county of New Castle and State of Delaware, have invented a certain new and useful Process of Making Propellant Powder, of which the following is a specification.

My invention relates to a process of producing explosives of an advantageous character, and more particularly to the production of propellant powders of the progressive type, that is to say, powders which have been so treated as to provide a lower initial pressure without reducing the velocity of the projectile. My invention is applicable to the various kinds of rifle and cannon powders.

The object of my invention is to provide a process of producing powders of this type which do not have the disadvantage of previous processes of producing powders containing coatings on the outside thereof but not impregnating the surface of the same, that is to say, the great difficulty of ignition which often resulted in hang fires.

Another object of my invention is to provide a process by which a powder is obtained which will produce considerably less erosion in rifle linings than previous powders.

A further object is to provide a process by means of which the surface of the powder grains may be effectively impregnated with a deterrent material which is not an explosive in such a manner that the grains are prevented from adhering to one another, as well as to secure more uniform impregnation of the grains by the coating materials than hitherto.

The deterrent materials which may be used in my process are particularly the dialkyldiarylureas, such as dimethyldiphenylurea,  $\text{CO}(\text{N}(\text{CH}_3)\text{C}_6\text{H}_5)_2$ ; diethyldiphenylurea,  $\text{CO}(\text{N}(\text{C}_2\text{H}_5)\text{C}_6\text{H}_5)_2$ ; methylethyldiphenylurea,  $\text{N}(\text{CH}_3)(\text{C}_6\text{H}_5)\text{CO.N}(\text{C}_2\text{H}_5)\text{C}_6\text{H}_5$ , etc., these ureas having in general a solvent or colloidizing action on nitrocellulose and the property of penetrating and impregnating the powder grain when heated with the latter in the presence of water to a temperature of not more than  $100^\circ \text{C}$ .

One object of my invention is especially to provide a process by means of which a

deterrent material such as dimethyldiphenylurea that is not explosive, which, because of its low volatility and good stability, as well as other properties would be suitable for surface impregnation of the smokeless powder grains, but which has such a high melting point that it could not be used in a melted condition to impregnate the surface of the powder grains because such high temperature would affect the stability of the powder, can be used because of the fact that it can be applied at even lower temperatures than its melting point, with the aid of hot water, as the presence of the water causes it to melt below the temperatures at which it would otherwise melt.

The object of my invention is furthermore to provide a process which is an improvement over the process as set forth in the application of Alfred L. Broadbent and myself upon the process of making propellant powder, Serial No. 109,249, filed July 14, 1916.

Further objects of my invention will appear from the detailed description thereof contained hereinafter.

While my invention is capable of embodiment in many different forms, for the purpose of illustration I shall describe only certain ways of carrying out my invention hereinafter.

For example, 100 parts by weight of nitrocellulose powder grains are introduced into a revolving mixing drum of any desired character, which may or may not be provided with longitudinally directed ribs on the interior cylindrical surface. Thereafter, I introduce into the drum 3 parts by weight of dimethyldiphenylurea, after which the entire mass is covered with water. The dimethyldiphenylurea may be practically pure, having a melting point between  $120^\circ$  and  $121^\circ \text{C}$ , but preferably I use a commercial dimethyldiphenylurea containing some impurities, and melting at  $110^\circ \text{C}$ , or over. After the materials in the drum have been thoroughly mixed, that is to say in from five to ten minutes, heat is applied in any suitable manner as by injecting steam into the drum or into a jacket thereon, while the temperature is gradually raised to between  $80^\circ \text{C}$  and  $100^\circ \text{C}$ , and preferably to between  $85$  and  $90^\circ \text{C}$ . This will be sufficient in the presence of the water to melt

or soften the dimethyldiphenylurea. Inasmuch as the dimethyldiphenylurea is a solvent of nitrocellulose, it colloids the nitrocellulose and impregnates the surface of the grains. The temperature of 85 to 90° C. is maintained for about thirty minutes, as this is usually sufficient to impregnate the powder with the dimethyldiphenylurea and to cause the latter substance to be no longer visible on the surface of the grains. However, the impregnation is not complete in this period of time, so in order to render it complete the materials are removed to a stationary tank of hot water at a temperature between 80 and 100° C. and preferably between 85 and 90° C., where they remain for a period amounting approximately to twenty-four hours. After this the powder grains are removed and dried. The impregnation is completed in this manner and at the temperature referred to notwithstanding the fact that the dimethyldiphenylurea of the grade used might melt for example at 115° C.

25 A nitrocellulose powder before having been impregnated as above, will give in a military rifle a muzzle velocity of 2,700 feet per second and a mean pressure of 49,000 pounds per square inch, with a charge 30 weighing forty-five grains, while a sample of the powder impregnated as above, will give the same muzzle velocity with a mean pressure of only 40,000 to 42,000 pounds per square inch, with a charge weighing 47-48 grains. The difference in the erosive effect of the two powders is even more marked, as the erosion by the impregnated powder is only one-fourth to one-third that of the powder which has not been impregnated.

35 40 The proportions in the above mixture may be varied through wide limits. For example, three parts by weight of dimethyl-diphenylurea may be used, but any amount varying from one to ten parts by weight 45 may be used according to the ballistic result desired.

When the deterrent material employed is diethyldiphenylurea, which has a melting point of 79° C., the temperature of the water in the above described process is maintained between 65 and 70° C. In the case of methylethyldiphenylurea, with a melting point of 57-58° C., the water is maintained at a temperature between 50 and 60° C. In 55 other respects the conditions of operation are about the same.

While I have described my invention above in detail, I wish it to be understood that many changes may be made therein 60 without departing from the spirit of the invention.

I claim:—

1. The process which comprises impregnating the surface of an explosive grain 65 insoluble in water with a deterrent material,

all of the deterrent material used having a melting point above 100° C. and being substantially insoluble in water, by subjecting the grain, while intimately mixed with said deterrent material, to treatment with hot 70 water.

2. The process which comprises impregnating the surface of an explosive grain insoluble in water with a deterrent material, all of the deterrent material used being non-explosive and substantially insoluble in 75 water, by subjecting the grain, while intimately mixed with said deterrent material, to treatment with hot water.

3. The process which comprises impregnating the surface of an explosive grain insoluble in water with a deterrent material comprising essentially dimethyldiphenylurea, all of the deterrent material used being substantially insoluble in water, and having a 80 melting point above 100° C., by subjecting the grain, while intimately mixed with said deterrent material, to treatment with hot water.

4. The process which comprises impregnating the surface of an explosive grain insoluble in water with dimethyldiphenylurea as the sole deterrent, by subjecting the grain, while intimately mixed with said dimethyl-diphenylurea, to treatment with hot water. 90

5. The process which comprises impregnating the surface of an explosive grain insoluble in water with a deterrent material, all of the deterrent material used having a melting point above 100° C. and being substantially insoluble in water, by subjecting the grain, while intimately mixed with said deterrent material, to treatment with hot water, at a temperature below the melting 100 point of the deterrent material. 105

6. The process which comprises impregnating the surface of an explosive grain insoluble in water with a deterrent material all of the deterrent material used being non-explosive and substantially insoluble in 110 water, by subjecting the grain, while intimately mixed with said deterrent material, to treatment with hot water, at a temperature below the melting point of the deterrent material. 115

7. The process which comprises impregnating the surface of an explosive grain insoluble in water with a deterrent material comprising essentially dimethyldiphenylurea, all of the deterrent material used being substantially insoluble in water, and having a melting point above 100° C., by subjecting the grain, while intimately mixed with said deterrent material, to treatment with hot water, at a temperature below the 120 melting point of the deterrent material. 125

8. The process which comprises impregnating the surface of an explosive grain insoluble in water with dimethyldiphenylurea as the sole deterrent, by subjecting the grain, 130

while intimately mixed with said dimethyl-diphenylurea, to treatment with hot water, at a temperature below the melting point of the dimethyldiphenylurea.

5 9. The process which comprises impregnating the surface of a nitrocellulose powder grain insoluble in water with a deterrent material, all of the deterrent material used having a melting point above 100° C. and 10 being substantially insoluble in water, by subjecting the grain, while intimately mixed with said deterrent material, to treatment with hot water, at a temperature below the melting point of the deterrent material.

15 10. The process which comprises impregnating the surface of a nitrocellulose powder grain insoluble in water with a deterrent material, all of the deterrent material used being not explosive and substantially 20 insoluble in water, by subjecting the grain, while intimately mixed with said deterrent material, to treatment with hot water, at a temperature below the melting point of the deterrent material.

25 11. The process which comprises impregnating the surface of a nitrocellulose powder grain insoluble in water with dimethyl-diphenylurea as the sole deterrent by subjecting the grain, while intimately mixed 30 with said dimethyldiphenylurea, to treatment with hot water, at a temperature below the melting point of the dimethyldiphenylurea.

35 12. The process of treating nitrocellulose powder grains which consists in treating with hot water said grains intimately mixed with a dialkyldiarylurea having a colloidizing action on said grains and capable of impregnating said grains in the presence of water 40 maintained at a temperature of less than 100%.

13. The process of treating nitrocellulose

powder grains which consists in treating with hot water said grains intimately mixed with a methylalkyldiphenylurea.

45

14. The process of treating nitrocellulose powder grains which consists in subjecting said grains while intimately mixed with a deterrent material composed of a dialkyl-diarylurea to the action of a hot liquid 50 which is chemically inert with respect to said grains and said deterrent material, and in which said grains and said deterrent material are insoluble.

15. The process of treating nitrocellulose powder grains which comprises subjecting said grains while intimately mixed with a deterrent material, all of the material used being not explosive, to the action of a hot liquid 55 which is chemically inert with respect to said grains and said deterrent material, and in which said grains and said deterrent material are insoluble.

60

16. The process of treating nitrocellulose powder grains which consists in subjecting said grains while intimately mixed with dimethyldiphenylurea to the action, at a temperature between 80 and 100° C., of a liquid 65 which is chemically inert with respect to said grains and said dimethyldiphenylurea, and in which said grains and said dimethyldiphenylurea are insoluble.

70

17. The process of treating nitrocellulose powder grains which consists in subjecting said grains while intimately mixed with a deterrent material composed of a dialkyl-diarylurea to the action, at a temperature 75 below 100° C., of a liquid which is chemically inert with respect to said grains and said deterrent material, and in which said grains and said deterrent material are insoluble.

80

In testimony whereof I affix my signature.  
RICHARD GEORGE WOODBRIDGE, Jr.